

Patented Aug. 24, 1926.

## UNITED STATES PATENT OFFICE.

DARCY VAN DER WANT AND MARTINUS PETRUS ANTONIUS BOUMAN, OF ARNHEM,  
NETHERLANDS, ASSIGNORS TO NAAMLOOZE VENNOOTSCHAP NEDERLANDSCHE  
KUNSTZIJDEFABRIEK, OF ARNHEM, NETHERLANDS.

## MANUFACTURE OF ARTIFICIAL PRODUCTS FROM VISCOSE.

No Drawing. Application filed March 4, 1926, Serial No. 92,364, and in Germany March 5, 1925.

Our invention refers to improvements in the manufacture of artificial products. 50

The usual precipitating baths in the manufacture of artificial products from viscose, such as fibres, ribbons, straw and the like, contain a salt in addition to an acid, usually sulphuric acid; for example, sodium sulphate, magnesium sulphate and ammonium sulphate are salts which have been proposed 10 for this purpose.

Our present invention is based on the discovery that salts of the bivalent metals (other than zinc) of the group commonly referred to in analytical work as the "ammonium sulphide" group, that is to say, of bivalent metals (other than zinc) whose sulphides are not precipitated in presence of an acid, have a specific influence in the precipitating bath on cellulose hydrate fibres. 20 By our present invention the acid precipitating bath in the manufacture of artificial products from viscose contains a salt of such a metal, with or without the addition of another salt or salts or other additions, such 25 as glucose, commonly used in the process.

The artificial products obtained by our invention have a very great affinity for dye-stuffs, and can therefore be dyed in deep shades; also, owing to an equalizing action 30 which the salts in question exert on the fibre, dyeings produced on the artificial products obtained according to our invention are more even. We have further found that the salts of the bivalent metals, other 35 than zinc, whose sulphide is not precipitated in presence of an acid and whose atomic weight lies between 57 and 60, and preferably between 58,5 and 59,2, such as nickel and cobalt, are best suitable for the purpose we have in view. 40

Even a small quantity of the salt is sufficient for obtaining the desired effect, the effect being roughly proportional to the quantity of the added metal salt in the bath.

45 A bath containing one per cent of nickel sulphate produces a very good effect. The nickel sulphate need not be added to the bath as such, but may be formed in the

bath by the addition of another suitable nickel salt.

As a preferred embodiment of our invention the following example of a spinning bath is given; it must be understood, however, that our invention is in no way limited to the substances or quantities specified, as 55 other known spinning baths with additions according to our invention have proved to be very suitable for carrying out our invention.

10 parts by weight of sulphuric acid. 60

8 parts by weight of sodium sulphate.

16 parts by weight of magnesium sulphate.

1 part by weight of nickel sulphate.

Instead of nickel sulphate, other nickel 65 compounds may be used and also for instance cobalt nitrate; although the addition of a zinc salt to the precipitating bath does not form per se a part of our invention, a zinc salt may be present in the bath in addition to the nickel or other metallic salt 70 used according to our invention.

We claim:

1. A process of manufacturing artificial products from viscose consisting in precipitating the viscose solution in a spinning bath containing in addition to the usual spinning bath constituents at least one salt of a bivalent metal the atomic weight of which lies between 57 and 60 and whose sulphide is not precipitated in presence of an acid. 75

2. A process of manufacturing artificial products from viscose consisting in precipitating the viscose solution in a spinning 85 bath containing in addition to the usual spinning bath constituents at least one salt of a bivalent metal the atomic weight of which lies between 58,5 and 59,2 and whose sulphide is not precipitated in presence of 90 an acid.

In testimony whereof we affix our signature.

DARCY VAN DER WANT.  
M. P. A. BOUMAN.